

## UNITED STATES PATENT OFFICE.

GUSTAF AXEL HELLSTRAND, OF BUTTE, MONTANA.

## DIFFERENTIAL FLOTATION OF ORES.

No Drawing.

Application filed June 22, 1922. Serial No. 570,231.

*To all whom it may concern:*

Be it known that I, GUSTAF AXEL HELLSTRAND, a subject of the King of Sweden, residing at Butte, in the county of Silver Bow, State of Montana, have invented certain new and useful Improvements in Differential Flotation of Ores; and I do hereby declare the following to be a full, clear, and exact description of the invention, such as will enable others skilled in the art to which it appertains to make and use the same.

This invention relates to the concentration of ores by flotation, and more particularly to the differential flotation of mixed sulfide ores. The invention has for its object the provision of an improved method of concentrating mixed or complex sulfide ores by differential flotation. More particularly, the invention aims to provide an improved method of concentrating by differential flotation a mixed or complex sulfide ore containing zinc sulfide or blende associated with other metallic sulfides.

The complex or mixed sulfide ores, such, for example, as an ore carrying sulfides of lead, zinc, copper and iron, have offered many difficulties to treatment by gravity concentration as well as by flotation, and in the case of many ores of this type it has heretofore been practically impossible to make an economic separation of the various metalliferous constituents of the ore from one another.

The present invention contemplates an improved method of treating complex or mixed sulfide ores containing zinc sulfide associated with one or more other metallic sulfides, such as iron, lead and copper sulfides, whereby such other metallic sulfide or sulfides are differentially separated by flotation from the zinc sulfide. Such a complex or mixed sulfide ore may also carry precious metallic values, particularly silver as metallic silver or as a simple sulfide or as one of the many forms of silver minerals. In accordance with the method of the invention, any such precious metallic values in the ore pass in substantial amount along with the aforementioned other metallic sulfides and are thus separated from the zinc sulfide in the ore.

The object of differential flotation in the treatment of a complex or mixed sulfide ore of the aforementioned character is the economic advantage resulting from the separa-

tion of the valuable minerals in the ore. It is desirable in treating such a mixed sulfide ore by differential flotation to make:

(1) A lead product free from zinc, 60

(2) A zinc product free from lead, iron and copper

(3) A segregation of copper and iron with the lead rather than with the zinc, particularly if they carry precious values, 65

(4) A segregation of the silver and gold with the copper-iron-lead product rather than with the zinc product,

(5) A tailing free from valuable minerals. 70

I have discovered that an alkali or alkali-earth sulfide, such, for example, as sodium sulfide, when present in an ore pulp in the relatively small amount hereinafter specified, very advantageously promotes the differential separation by flotation of the metalliferous values in a mixed sulfide ore. Thus, in accordance with the present invention the mixed sulfide ore is appropriately treated with sodium monosulfide or with one of the polysulfides of sodium, or with 80 any other alkali or alkali-earth sulfide, and the thus treated ore is subsequently subjected to a flotation operation in the course of which the sulfides of lead and/or iron and/or copper and/or silver and/or gold are 85 selectively or differentially removed from the ore pulp in the overflow froth, leaving behind in the ore pulp the greater part of the zinc sulfide present in the ore. In other words, the treatment of the ore pulp with 90 the relatively small amount of an alkali or alkali-earth sulfide contemplated by the present invention substantially inhibits the flotation of zinc sulfide while permitting the flotation of the other metallic sulfides present in the ore. 95

I am well aware that sodium monosulfide and polysulfides are recognized flotation reagents and that their use has heretofore been suggested in the flotation of oxidized 100 minerals (such as lead and copper carbonates) not otherwise amenable to flotation without the use of the sodium sulfide. Sodium sulfide has also been used, I believe, in the flotation of various sulfide minerals 105 refractory to such treatment because of surface oxidation. The object of using sodium monosulfide or sodium polysulfides in such cases is to obtain a sulfidizing action on the oxidized or partially oxidized minerals, thus 110 permitting the application of flotation to the recovery of minerals which otherwise are

not amenable to flotation treatment. I am also aware that it has heretofore been proposed to effect differential flotation of mixed sulfide ores by submitting such ores to 5 flotation separation in a circuit containing in solution from 0.1% to 1% of a sulfide of an alkali metal or earth. As contrasted with these prior suggestions of the use in the flotation of ores of an alkali metal or earth 10 sulfide, my present invention contemplates an improvement in the differential flotation of mixed sulfide ores involving the preliminary treatment of the mixed sulfide ore with a relatively small amount of an alkali or 15 alkali-earth sulfide, as for example, from about one to seven pounds of sodium sulfide per ton of ore at a pulp dilution of about four parts of water to one part of ore, by weight.

20 The general procedure in carrying out the process of the invention is as follows: Commercial crude sodium sulfide equivalent to from about one to seven pounds of sodium sulfide per ton of ore is added to the mixed 25 sulfide ore, preferably in the grinding mill, along with about one-tenth to one pound per ton of ore of suitable oil such as coal tar creosote, or other equivalent flotation reagent. The amount of sodium sulfide will 30 vary with the nature of the ore and the pulp dilution at which the differential flotation is carried out. The ore is ground fine enough to free the minerals, and also fine enough for flotation.

35 The differential result can be obtained with any reasonable pulp density, for example, four parts of water to one part of ore, by weight, but for a given ore the amount of sodium sulfide per ton of ore 40 will be relatively smaller with low pulp dilution than with high pulp dilution. A constant pulp density is essential for the best differential results after the reagents have been properly proportioned to a given 45 pulp density. The ore pulp is now subjected to treatment in a flotation machine in order to separate the sulfides of lead, iron and copper from the zinc sulfide. Any type of flotation machine commonly used in the art 50 may be employed for this purpose. A small amount of additional oil, such as cresylic acid or pine oil, may be added in the flotation machine. However, an excess of oil is to be avoided because any excess 55 of oil tends to destroy the differential results. The differential flotation is usually made in cold pulp.

60 The ore pulp remaining after the aforementioned differential flotation treatment contains the greater part of the zinc sulfide present in the original ore. This remaining ore pulp is now subjected to a further flotation operation for the removal therefrom of the zinc sulfide. This subsequent flotation 65 for removing zinc sulfide from the ore

pulp may be carried out under either alkaline or acid conditions. In alkaline flotation, I have obtained good results with one to two pounds of oil mixtures (consisting of coal tar oil, coal tar creosote and pine oil), a 70 fraction of a pound to two pounds of caustic soda or one to three pounds of sodium carbonate, and five-tenths to one pound of copper sulfate, per ton of ore. In acid flotation, good results have been obtained with a 75 fraction of a pound of pine oil, per ton of ore, and sulfuric acid sufficient to make the pulp slightly acid. The ore pulp, with the additional reagents above mentioned, is now subjected to a second flotation operation 80 and a froth concentrate is obtained containing substantially all of the zinc sulfide present in the ore. With acid pulp the flotation of the zinc sulfide is facilitated by heating the ore pulp to about 95° F. The 85 zinc flotation under alkaline conditions is usually carried out in cold pulp.

A departure from the above procedure 90 may be desirable in the treatment of certain ores. For example, the sodium sulfide may be introduced into the ore pulp at different stages during the process in addition to the amount added in the grinding mill, or the entire amount of this reagent may be added 95 in the flotation machine, or to the ore pulp just prior to its introduction into the flotation machine. Moreover, all of the oil may be added in the grinding mill, or all may be added in the flotation machine or to the ore 100 pulp just prior to its introduction into the flotation machine.

The method of the invention has a wide field of application and has given excellent economical results in the treatment of a large number of mixed or complex sulfide 105 ores in which problems of differential separation were presented. The following specific examples will clearly indicate the wide applicability of the invention. In plant practice commercial crude sodium sulfide, 110 usually of a grade equivalent to 60% to 62% sodium sulfide, is generally used. In laboratory tests, however, I have used both the crude and chemically pure sodium sulfide. The difference in these two products, as respects the present invention, is merely in the 115 relative soluble sulfide content, one pound of 60% commercial crude sodium sulfide being equivalent to 0.6 pound sodium sulfide.

#### EXAMPLE No. 1—ORE "A."

The ore was ground wet to pass 65 mesh, along with four pounds of commercial crude sodium sulphide (62% sodium sulphide) and about 0.1 pound of an oil mixture (consisting of 90% coal tar creosote and 125 10% pine oil), per ton of ore.

The lead-iron concentrate was obtained by the addition of about 0.15 pound, per ton of ore, of the oil mixture to an ore pulp 130

of three parts of water to one part of ore, by weight, and subjecting the ore pulp to a flotation operation.

The remaining ore pulp was then slightly acidified with sulphuric acid and heated to 95° F. and subjected to a further flotation operation with additional amount of oil mixture to obtain the zinc concentrate.

10

## Assay.

| Product.          | Wt. per cent of total. | Per cent Cu. | Oz. Ag. | Per cent insol. | Per cent Fe. | Per cent Zn. | Per cent Pb. |
|-------------------|------------------------|--------------|---------|-----------------|--------------|--------------|--------------|
| 15 Head.....      | 100.0                  | 0.18         | 6.7     | 66.4            | 1.7          | 16.2         | 2.02         |
| Pb.-Fe. conc..... | 7.1                    | 1.13         | 32.8    | 8.6             | 19.6         | 13.1         | 22.30        |
| Zn. conc.....     | 23.3                   | 0.45         | 16.5    | 5.5             | 0.4          | 60.2         | 1.34         |
| Zn. middling..... | 6.7                    | .....        | 5.1     | .....           | 0.6          | 14.3         | 0.76         |
| Tailing.....      | 62.9                   | .....        | 0.3     | .....           | 0.25         | 0.4          | 0.12         |
| 20 Total.....     | 100.0                  | .....        | .....   | .....           | .....        | .....        | .....        |

TABLE No. 1A—RECOVERY—CALC. TO 100%.

| Product.          | Per cent of total. |       |       |       |
|-------------------|--------------------|-------|-------|-------|
|                   | Ag.                | Fe.   | Zn.   | Pb.   |
| Head.....         | 100.0              | 100.0 | 100.0 | 100.0 |
| Pb.-Fe. conc..... | 34.7               | 82.8  | 5.8   | 78.4  |
| Zn. conc.....     | 57.4               | 5.5   | 88.8  | 15.4  |
| Zn. middling..... | 5.1                | 2.4   | 5.9   | 2.5   |
| Tailing.....      | 2.8                | 9.3   | 1.5   | 3.7   |
| Total.....        | 100.0              | 100.0 | 100.0 | 100.0 |

The zinc concentrate in the foregoing example was obtained by acid flotation.

The following tabulation shows the lead-iron and zinc concentrates combined in a single product in order to represent the results of a collective flotation process:

| Product.                            | Assay.                 |              |         |                 |              |              |              |
|-------------------------------------|------------------------|--------------|---------|-----------------|--------------|--------------|--------------|
|                                     | Wt. per cent of total. | Per cent Cu. | Oz. Ag. | Per cent insol. | Per cent Fe. | Per cent Zn. | Per cent Pb. |
| 5 Pb.-Fe. and Zn. conc. comb'd..... | 30.4                   | 0.61         | 20.3    | 6.2             | 4.9          | 49.2         | 6.24         |
| Zn. mid.....                        | 6.7                    | .....        | 5.1     | .....           | 0.6          | 14.3         | 0.76         |
| Tailing.....                        | 62.9                   | .....        | 0.3     | .....           | 0.25         | 0.4          | 0.12         |
| 50 Total.....                       | 100.0                  | .....        | .....   | .....           | .....        | .....        | .....        |

TABLE No. 2A—RECOVERY—CALC. TO 100%.

| Product.                        | Per cent of total. |       |       |       |
|---------------------------------|--------------------|-------|-------|-------|
|                                 | Ag.                | Fe.   | Zn.   | Pb.   |
| Pb.-Fe. and Zn. conc. comb'd .. | 92.1               | 88.3  | 92.6  | 93.8  |
| Zn. mid.....                    | 5.1                | 2.4   | 5.9   | 2.5   |
| Tailing.....                    | 2.8                | 0.3   | 1.5   | 3.7   |
| Total.....                      | 100.0              | 100.0 | 100.0 | 100.0 |

The advantages of the method of the invention applied to this particular ore (A) may be summed up as follows:

(1) A segregation into an economic product of comparatively small amounts of lead, iron and copper sulfides in the ore;

(2) The elimination of these sulfides assures a high grade zinc product;

(3) A segregation of an appreciable portion of the silver in the differential product, which may be a matter of decided economic advantage, since payment for silver in such differential product is higher than in the zinc product;

(4) A change to acid condition for zinc flotation since this is the most favorable condition for the maximum zinc recovery.

80

## EXAMPLE No. 2—ORE "B."

The ore was ground wet to pass 65 mesh, along with seven pounds of commercial crude sodium sulphide (62% sodium sulphide) and about 0.1 pound of coal tar creosote, per ton of ore.

The lead-iron concentrate was obtained by adding about 0.1 pound of pine oil, per ton of ore, to an ore pulp of four parts of water to one part of ore, by weight, and subjecting the ore pulp to a flotation operation.

The zinc concentrate was obtained by subjecting the remaining ore pulp to a further flotation operation with two pounds of sodium carbonate, 0.75 pound of copper sulphate, two pounds of an oil mixture (consisting of coal tar oil, coal tar creosote and pine oil), per ton of ore.

95

100

## Assay.

| Product.          | Wt. per cent of total. | Oz. Ag. | Per cent insol. | Per cent Fe. | Per cent Zn. | Per cent Pb. |
|-------------------|------------------------|---------|-----------------|--------------|--------------|--------------|
| Head.....         | 100.0                  | 12.6    | 65.3            | 3.3          | 14.7         | 1.34         |
| Pb.-Fe. conc..... | 10.3                   | 37.1    | 10.8            | 30.3         | 6.0          | 12.40        |
| Zn. conc.....     | 21.9                   | 37.9    | 3.8             | 0.4          | 60.0         | 0.27         |
| Zn. mid.....      | 3.4                    | 7.1     | 75.2            | 0.6          | 11.5         | 0.05         |
| Tailing.....      | 64.4                   | 0.4     | .....           | 0.1          | 0.9          | Tr.          |
| Total.....        | 100.0                  | .....   | .....           | .....        | .....        | .....        |

105

TABLE No. 1B—RECOVERY—CALC. TO 100%.

| Product.          | Per cent of total. |       |       |       |
|-------------------|--------------------|-------|-------|-------|
|                   | Ag.                | Fe.   | Zn.   | Pb.   |
| Head.....         | 100.0              | 100.0 | 100.0 | 100.0 |
| Pb.-Fe. conc..... | 30.3               | 94.8  | 4.2   | 95.4  |
| Zn. conc.....     | 65.8               | 2.8   | 89.2  | 4.4   |
| Zn. mid.....      | 1.9                | 0.6   | 2.7   | 0.2   |
| Tailing.....      | 2.0                | 1.8   | 3.9   | ..... |
| Total.....        | 100.0              | 100.0 | 100.0 | 100.0 |

110

115

120

125

In the following tabulation the lead-iron and zinc concentrates have been combined

130

to present the products obtained by a collective flotation process:

| 5  | Product.                       | Assay.                 |         |                 |              |              |              |
|----|--------------------------------|------------------------|---------|-----------------|--------------|--------------|--------------|
|    |                                | Wt. per cent of total. | Oz. Ag. | Per cent insol. | Per cent Fe. | Per cent Zn. | Per cent Pb. |
| 10 | Pb.-Fe. and Zn. conc's comb'd. | 32.2                   | 37.7    | 6.0             | 9.9          | 42.7         | 4.15         |
|    | Zn. middling                   | 3.4                    | 7.1     | 75.2            | 0.6          | 11.5         | 0.05         |
|    | Tailing                        | 64.4                   | 0.4     | -----           | 0.1          | 0.9          | Tr.          |
|    | Total                          | 100.0                  |         |                 |              |              |              |

15 TABLE NO. 1C—RECOVERY—CALC. TO 100%.

| 20 | Product.                       | Per cent of total. |       |       |       |
|----|--------------------------------|--------------------|-------|-------|-------|
|    |                                | Ag.                | Fe.   | Zn.   | Pb.   |
| 25 | Pb.-Fe. and Zn. conc's comb'd. | 98.1               | 97.6  | 93.4  | 69.8  |
|    | Zn. middling                   | 1.9                | 0.6   | 2.7   | 0.2   |
|    | Tailing                        | 2.0                | 1.8   | 3.9   | ----- |
|    | Total                          | 100.0              | 100.0 | 100.0 | 100.0 |

The advantages of the method of the invention in the differential flotation of the metalliferous values in this ore (B) is clearly illustrated in the foregoing data. 30 In the foregoing example, the zinc flotation was carried out under alkaline conditions. There are a number of alkaline flotation processes which will give a high grade zinc product, usually by dropping the iron sulfide in the tailing; but in mill practice the zinc lost in the tailing under this condition is higher because zinc flotation is carried on under differential conditions in contrast to intense flotation 35 conditions essential to zinc recovery. 40

#### EXAMPLE NO. 3—ORE "C."

45 The preliminary treatment of the ore in the grinding operation was the same as in example No. 1.

The silver concentrate was obtained under the same condition as set forth for the 50 lead-iron concentrate in example No. 1.

The zinc flotation was carried out as in example No. 1, except that the concentrate was not retreated.

#### 55 Assay.

| 60        | Product. | Wt. per cent of total. | Per cent Cu. | Oz. Ag. | Oz. Au. | Per cent insol. | Per cent Fe. | Per cent Zn. |
|-----------|----------|------------------------|--------------|---------|---------|-----------------|--------------|--------------|
| Head      | .....    | 100.0                  | 0.44         | 33.4    | 0.05    | 54.8            | 2.0          | 25.1         |
| Ag. conc. | .....    | 8.4                    | 2.72         | 288.3   | 0.22    | 8.8             | 22.2         | 19.6         |
| Zn. conc. | .....    | 39.0                   | 0.51         | 22.8    | 0.05    | 6.0             | 0.3          | 59.8         |
| Tailing   | .....    | 52.6                   | 0.02         | 0.3     | 0.003   | -----           | 0.1          | 0.4          |
| Total     | .....    | 100.0                  |              |         |         |                 |              |              |

TABLE NO. 1C—RECOVERY—CALC. TO 100%.

| Product.  | Per cent of total. |       |       |       |       |
|-----------|--------------------|-------|-------|-------|-------|
|           | Cu.                | Ag.   | Au.   | Fe.   | Zn.   |
| Head      | 100.0              | 100.0 | 100.0 | 100.0 | 100.0 |
| Ag. conc. | 52.0               | 72.1  | 53.8  | 91.6  | 6.6   |
| Zn. conc. | 45.5               | 26.6  | 39.0  | 5.9   | 92.6  |
| Tailing   | 2.5                | 1.3   | 7.2   | 2.5   | 0.8   |
| Total     | 100.0              | 100.0 | 100.0 | 100.0 | 100.0 |

70

75

Undoubtedly some silver exists in association with the principal sulfide minerals in this ore (C); but the indications are that silver occurs largely as distinct silver minerals.

Acid zinc flotation followed differential flotation in the foregoing example.

#### EXAMPLE NO. 4—ORE "D."

85

The preliminary treatment of the ore in the grinding operation was the same as in example No. 2.

The copper concentrate was obtained under the same condition as set forth for the lead-iron concentrate in example No. 2.

The zinc flotation was carried out as in example No. 2.

In the zinc flotation, in examples Nos. 1, 95 2 and 4, the first or rougher, concentrate obtained was subjected to another flotation treatment (or cleaning operation) and the tailing from this cleaning operation is shown as zinc middling.

100

#### Assay.

| Product.  | Wt. per cent of total. | Per cent Cu. | Oz. Ag. | Per cent insol. | Per cent Fe. | Per cent Zn. |
|-----------|------------------------|--------------|---------|-----------------|--------------|--------------|
| Head      | 100.0                  | 2.03         | 25.7    | 65.3            | 3.3          | 13.0         |
| Cu. conc. | 10.1                   | 9.42         | 109.0   | 10.6            | 15.2         | 25.8         |
| Zn. conc. | 13.3                   | 1.36         | 29.0    | 6.1             | 1.2          | 57.6         |
| Zn. mid.  | 3.9                    | 0.79         | 8.2     | -----           | 2.8          | 5.9          |
| Tailing   | 63.7                   | 0.08         | 1.1     | -----           | 0.2          | 0.3          |
| Total     | 100.0                  |              |         |                 |              |              |

105

TABLE NO. 1D—RECOVERY—CALC. TO 100%.

| Product.  | Per cent of total. |       |       |       |
|-----------|--------------------|-------|-------|-------|
|           | Cu.                | Ag.   | Fe.   | Zn.   |
| Head      | 100.0              | 100.0 | 100.0 | 100.0 |
| Cu. conc. | 87.2               | 81.0  | 87.9  | 37.9  |
| Zn. conc. | 8.8                | 15.0  | 4.9   | 58.8  |
| Zn. mid.  | 1.5                | 1.3   | 3.3   | 1.8   |
| Tailing   | 2.5                | 2.7   | 3.9   | 1.5   |
| Total     | 100.0              | 100.0 | 100.0 | 100.0 |

110

115

#### EXAMPLE NO. 5—ORE "E."

120

125

The ore was ground wet to pass 65 mesh. The lead concentrate was obtained with the addition of three pounds of commercial

130

5 crude sodium sulphide (62% sodium sulphide) and about one pound of an oil mixture (consisting of 90% coal tar creosote and 10% pine oil), per ton of ore, to an ore pulp of two and half parts of water to one part of ore, by weight, and subjecting the ore pulp to a flotation operation.

## Assay.

| 10 Product.      | Wt. per cent of total. | Per cent insol. | Per cent Fe. | Per cent Zn. | Per cent Pb. |
|------------------|------------------------|-----------------|--------------|--------------|--------------|
| Head.....        | 100.0                  | 71.5            | 1.3          | 2.1          | 5.4          |
| 15 Pb. conc..... | 9.1                    | 14.5            | 2.0          | 7.9          | 58.6         |
| Tailing.....     | 90.9                   | .....           | 1.2          | 1.5          | 0.1          |
| Total.....       | 100.0                  | .....           | .....        | .....        | .....        |

TABLE NO. 1E—RECOVERY—CALC. TO 100%.

| 20 Product.   | Per cent of total. |       |       |
|---------------|--------------------|-------|-------|
|               | Fe.                | Zn.   | Pb.   |
| 25 Head.....  | 100.0              | 100.0 | 100.0 |
| Pb. conc..... | 14.3               | 34.6  | 88.3  |
| Tailing.....  | 85.7               | 65.4  | 1.7   |
| Total.....    | 100.0              | 100.0 | 100.0 |

30 The foregoing example shows a good recovery of lead in a high grade product.

## EXAMPLE No. 6—ORE "F."

35 The ore was ground wet to pass 65 mesh, along with six pounds of C. P. sodium sulphide and about 0.15 pound of coal tar creosote, per ton of ore.

40 The lead-iron concentrate was obtained by the addition of about 0.2 pound of an oil mixture (consisting of 25% pine oil and 75% cresylic acid) per ton of ore, to an ore pulp of four parts of water to one part of ore, by weight, and subjecting the ore pulp to a flotation operation.

45 The zinc concentrate was obtained by subjecting the remaining ore pulp to a further flotation operation, with the addition of one pound of sodium carbonate, 0.75 pound copper sulphate and about one pound of an oil mixture (consisting of 90% coal tar creosote and 10% pine oil), per ton of ore.

## Assay.

| 55 Product.       | Wt. Per cent of total. | Oz. Ag. | Per cent insol. | Per cent Fe. | Per cent Zn. | Per cent Pb. |
|-------------------|------------------------|---------|-----------------|--------------|--------------|--------------|
| 60 Head.....      | 100.0                  | 34.6    | 54.6            | 4.0          | 10.1         | 4.97         |
| Pb.-Fe. conc..... | 14.6                   | 169.8   | 5.8             | 16.9         | 13.5         | 28.92        |
| Zn. conc.....     | 15.8                   | 49.3    | 5.0             | 5.2          | 49.0         | 4.50         |
| Tailing.....      | 69.6                   | 5.0     | .....           | 0.9          | 0.5          | 0.05         |
| Total.....        | 100.0                  | .....   | .....           | .....        | .....        | .....        |

TABLE NO. 1F—RECOVERY—CALC. TO 100%.

| Product.          | Per cent of total. |       |       |       |
|-------------------|--------------------|-------|-------|-------|
|                   | Ag.                | Fe.   | Zn.   | Pb.   |
| Head.....         | 100.0              | 100.0 | 100.0 | 100.0 |
| Pb.-Fe. conc..... | 71.6               | 63.0  | 19.6  | 85.0  |
| Zn. conc.....     | 18.4               | 21.0  | 77.0  | 14.3  |
| Tailing.....      | 10.0               | 16.0  | 3.4   | 0.7   |
| Total.....        | 100.0              | 100.0 | 100.0 | 100.0 |

The quantity of oil that may be used in carrying out the method of the invention with good differential results may be more or less than the amounts hereinbefore specified. Moreover, the method of the invention is not restricted to the use of sodium sulfide, but, on the contrary the differential results contemplated by the invention may be secured by other soluble sulfides and in particular by the polysulfides of sodium as well as by the sulfides of the other alkali metals and alkali-earth metals.

Chemically pure reagents are not essential for the satisfactory operation of the improved process of differential flotation contemplated by the invention. Thus, the invention may be successfully practiced with commercial crude sodium sulfide (also commercial crude sulfides of the other alkali and alkali-earth metals) containing impurities such as sulfites, hypo-sulfites, sulfates, carbonates, and other salts.

The essential feature in the improved method of the invention resides in the use of a soluble sulfide, such as sodium sulfide or an equivalent sulfide in proper amount and under proper conditions. Such soluble sulfide is generally used alone but may be used in conjunction with a weak base or with a very small amount of a strong base depending on the character of the ore. The effect of sodium sulfide (or other equivalent soluble sulfide) as a differential flotation reagent when employed in accordance with the present invention is exhibited (1) in the acceleration of the flotation of lead and/or iron and/or copper sulfides, (2) in the inhibition of the flotation of zinc sulfide, and (3) in the concentration of silver minerals in the differential product rather than in the zinc product.

The treatment of a mixed sulfide ore with the relatively small amount of an alkali or alkali-earth sulfide contemplated by the present invention secures certain advantageous results among which may be mentioned the production of a relatively stable and easily removed froth, which is an important factor from the standpoint of practical mill operation. Where the method of the invention is applied to the differential separation of lead sulfide from zinc sulfide,

the relatively small amount of alkali or alkali-earth sulfide employed insures satisfactory zinc flotation, especially if it is desired to carry on acid zinc flotation, where as the use of much larger amounts of the alkali or alkali-earth sulfide will unfavorably affect the zinc flotation due to the presence in the ore pulp of an appreciable quantity of hydrogen sulfide gas and other products formed by the action of sulfuric acid on the alkali or alkali-earth sulfide.

From the foregoing description and examples, it will be evident to those skilled in the art that the method of the invention provides an effective procedure for differentially separating from zinc sulfide certain other metallic sulfides associated with such zinc sulfide in a mixed or complex ore. In particular, the method of the invention is especially applicable to such differential flotation problems as the following:

- (1) The separation of lead sulfide from zinc sulfide;
- (2) The separation of iron sulfide (pyrite) from zinc sulfide;
- (3) The separation of copper sulfide (particularly chalcopyrite and bornite) from zinc sulfide, and
- (4) The separation of lead and copper sulfides (particularly chalcopyrite and bornite) from zinc sulfide.

I claim:

1. A process of concentrating by flotation an ore containing zinc sulfide and one or more other metallic sulfides, which comprises subjecting the ore to treatment with a soluble sulfide in amount, not exceeding about seven pounds per ton of ore, proportioned to effectively inhibit the flotation of zinc sulfide, and subjecting the so treated ore to a flotation operation in which the flotation of the zinc sulfide is in large part inhibited.

2. A process of concentrating by flotation an ore containing zinc sulfide and one or more other metallic sulfides, which comprises subjecting the ore to treatment with a soluble sulfide in amount, not exceeding about seven pounds per ton of ore, proportioned to effectively inhibit the flotation of zinc sulfide, subjecting the so treated ore to a flotation operation and thereby obtaining a concentrate containing a relatively high percentage of such other metallic sulfide or sulfides, and thereafter subjecting the remaining ore pulp to another flotation operation under appropriate conditions permitting the flotation of the zinc sulfide.

3. A process of concentrating by flotation an ore containing zinc sulfide associated with one or more other metallic sulfides and with minerals of the precious metals, which comprises treating the ore with a soluble

sulfide in an amount, not exceeding about seven pounds per ton of ore, proportioned to effectively inhibit the flotation of zinc sulfide, and subjecting the thus treated ore to a flotation operation and thereby obtaining a froth concentrate containing a relatively high percentage of the precious metals and said other metallic sulfide or sulfides while the flotation of the zinc sulfide is substantially inhibited.

4. A process of concentrating by flotation an ore containing lead sulfide and zinc sulfide, which comprises treating the ore with a soluble sulfide in amount, not exceeding about seven pounds per ton of ore, proportioned to effectively inhibit the flotation of the zinc sulfide, and subjecting the thus treated ore to a flotation operation and thereby obtaining a froth concentrate containing a relatively high percentage of the lead sulfide and inhibiting in large part the flotation of the zinc sulfide.

5. A process of concentrating by flotation an ore containing lead, copper, and zinc sulfides, which comprises treating the ore with a soluble sulfide in amount, not exceeding about seven pounds per ton of ore, proportioned to effectively inhibit the flotation of zinc sulfide, and subjecting the thus treated ore to a flotation operation and thereby obtaining a froth concentrate containing a relatively high percentage of the lead and copper sulfides and inhibiting in large part the flotation of the zinc sulfide.

6. A process of concentrating by flotation an ore containing lead, iron, copper, and zinc sulfides, which comprises treating the ore with a soluble sulfide in amount, not exceeding about seven pounds per ton of ore, proportioned to effectively inhibit the flotation of zinc sulfide, and subjecting the thus treated ore to a flotation operation and thereby obtaining a froth concentrate containing a relatively high percentage of the lead, iron, and copper sulfides and inhibiting in large part the flotation of the zinc sulfide.

7. A process of concentrating by flotation an ore containing iron and zinc sulfides, which comprises treating the ore with a soluble sulfide in amount, not exceeding about seven pounds per ton of ore, proportioned to effectively inhibit the flotation of zinc sulfide, and subjecting the thus treated ore to a flotation operation and thereby obtaining a froth concentrate containing a relatively high percentage of the iron sulfide and inhibiting in large part the flotation of the zinc sulfide.

8. A process of concentrating by flotation an ore containing copper and zinc sulfides, which comprises treating the ore with a soluble sulfide in amount, not exceeding

about seven pounds per ton of ore; proportioned to effectively inhibit the flotation of zinc sulfide, and subjecting the thus treated ore to a flotation operation and thereby obtaining a froth concentrate containing a relatively high percentage of the copper sul-

fide and inhibiting in large part the flotation of the zinc sulfide.

In testimony whereof I affix my signature.

GUSTAF AXEL HELLSTRAND.